

May 14, 1963

J. C. SIPLE

3,089,780

METHOD AND COMPOSITION FOR SHIELDING STEEL  
FROM MOLTEN COATING METAL

Filed May 4, 1961



INVENTOR.  
JAMES C. SIPLE

By *Donald G. Dalton*

Attorney

## 1

3,089,780

METHOD AND COMPOSITION FOR SHIELDING  
STEEL FROM MOLTEN COATING METALJames C. Siple, Mount Lebanon Township, Allegheny  
County, Pa., assignor to United States Steel Corpora-  
tion, a corporation of New Jersey

Filed May 4, 1961, Ser. No. 107,630

4 Claims. (Cl. 117—5.5)

This invention relates to the manufacture of sheet steel 10  
coated with protective metal on one side only.

As explained in Greene et al. Patent No. 2,894,850, a  
demand has arisen for steel sheets galvanized on one  
side only. These patentees disclose the coating of sheet  
steel on one side with a shielding layer of sodium alu-  
minate, before galvanizing by hot-dipping, to prevent the  
adherence of zinc to the surface previously coated with  
aluminate.

I have invented a novel composition for this purpose  
which has important advantages over sodium aluminate.  
In accordance with my invention, I form a slurry of mag-  
nesium oxide in a solution of an alkali-metal salt of meta-  
boric acid such as sodium metaborate. This provides an  
inexpensive yet effective shielding layer which is readily  
removable by washing with water after the zinc coating  
has been applied to one side of the sheet.

The essential steps of a typical example of my method  
are shown in the accompanying drawing which is a flow  
sheet of the method.

More specifically, my shielding composition is a slurry  
of fully calcined magnesium oxide in a solution of an  
alkali-metal metaborate. I prepare a mixture contain-  
ing from 3 to 20% sodium metaborate, for example, by  
weight, preferably about 6%, and from 12 to 28% of  
the oxide, by weight, preferably about 21%, and the  
balance water. This mixture, well stirred, is applied to  
one side of low-carbon sheet steel, containing less than  
0.75% silicon, preferably in strip form, in any convenient  
manner as by brushing, spraying or roller coating of  
which the latter is preferred. The coating is dried by  
mild heating after which the solid material remaining  
amounts to about 1 gram per square foot.

The steel is then passed through a galvanizing bath,  
preferably after a conventional continuous annealing  
treatment. After the galvanized strip is cooled in air,  
the shielded surface of the strip is scrubbed with water  
to remove the oxide-metaborate film. A light scrubbing  
is sufficient to remove the shielding coating, leaving the  
uncoated surface of the steel exposed throughout. The 50  
side of the steel sheet not coated with the oxide-metaborate  
film, of course, is uniformly coated with zinc as  
a result of passage through the galvanizing bath. If  
necessary, a gas flame is directed onto the shielded side  
of the steel as it emerges from the galvanizing bath, to  
remove any zinc particles which may be mechanically  
dragged out.

The invention has numerous advantages over prior  
practice. In the first place, the oxide-metaborate film

## 2

may be used successfully where continuous annealing oc-  
curs just before the galvanizing. Secondly, the shielding  
layer is composed of inexpensive materials, and may be  
easily applied and removed. It effectively prevents coat-  
ing by zinc on the shielded side and, when removed,  
leaves a steel surface suitable for welding, painting or  
other treatment. The shielding film is tightly adherent  
and abrasion-resistant so as to permit passing through  
the annealing process without damage. Thus the inven-  
tion may be utilized without altering conventional an-  
nealing and galvanizing practice.

Potassium metaborate and other alkali-metal meta-  
borates may be used in place of the sodium salt. Cal-  
cium oxide may be used instead of magnesium oxide, or  
a mixture of both. The shielding composition of my  
invention may also be used to prevent coating of steel  
with aluminum, tin and terne when immersed in molten  
baths thereof.

Although I have disclosed herein the preferred em-  
bodiment of my invention, I intend to cover as well any  
change or modification therein which may be made with-  
out departing from the spirit and scope of the invention.

I claim:

1. A composition for shielding steel from coating by  
metal when immersed in a molten bath thereof consist-  
ing essentially of a water slurry containing from 12 to  
28% by weight of an oxide selected from the group con-  
sisting of calcium oxide and magnesium oxide, and from  
3 to 20% by weight of an alkali-metal metaborate.

2. A composition as defined in claim 1 wherein the  
salt is sodium metaborate.

3. A composition for shielding steel from coating by  
metal when immersed in a molten bath thereof consisting  
essentially of a water slurry containing about 21% mag-  
nesium oxide by weight and about 6% of an alkali-metal  
metaborate by weight.

4. A method of shielding steel from coating by metal  
selected from the group consisting of aluminum, zinc,  
tin and terne, when immersed in a molten bath thereof,  
which comprises applying to the surface of the steel a  
water slurry consisting essentially of from 12 to 28% by  
weight of an oxide selected from the group consisting  
of calcium oxide and magnesium oxide, and from 3 to  
20% sodium metaborate by weight and drying the result-  
ing film, then immersing the steel in the bath.

## References Cited in the file of this patent

## UNITED STATES PATENTS

|           |               |               |
|-----------|---------------|---------------|
| 940,111   | Ackermann     | Nov. 16, 1909 |
| 2,343,158 | Scott         | Feb. 29, 1944 |
| 2,502,198 | Benner et al. | Mar. 28, 1950 |
| 2,618,530 | Gardner       | Nov. 18, 1952 |
| 2,858,235 | Rex           | Oct. 28, 1958 |
| 2,894,850 | Greene et al. | July 14, 1959 |
| 2,955,958 | Brown         | Oct. 11, 1960 |

## FOREIGN PATENTS

|         |               |             |
|---------|---------------|-------------|
| 725,778 | Great Britain | Mar. 9 1955 |
|---------|---------------|-------------|